

1

3,296,104

### ELECTRODEPOSITION OF ZINC FROM PYROPHOSPHATE SOLUTIONS

Frederick W. Eppensteiner, Woodbridge, N.J., assignor to Hanson-Van Winkle-Munning Company  
No Drawing. Filed Oct. 29, 1963, Ser. No. 319,666  
15 Claims. (Cl. 204—55)

This invention relates to the electrodeposition of bright zinc in an alkaline pyrophosphate bath containing an improved brightener composition. The invention is based on the discovery that certain organic compounds when incorporated in an alkaline pyrophosphate zinc bath in combination with various carbonyl compounds of the aldehyde and ketone types are capable of promoting the formation of excellent bright and uniformly smooth electrodeposits of zinc over a wide current density range. Moreover, the additives of this invention greatly improve the throwing power of the zinc pyrophosphate plating solution making it particularly suitable for barrel plating.

Alkaline solutions containing complex compounds of zinc and alkali metal pyrophosphates have been proposed as a replacement for the cyanide bath in electrodeposition of bright zinc, thereby eliminating the troublesome and costly disposal problem associated with the use of cyanide baths. Electrodeposition of zinc using the pyrophosphate bath, however, shows poor low current density coverage, lack of brightness and uniformity of the deposit. Attempts to overcome the deficiency of the bath by adding a few comparatively expensive additives such as ortho-hydroxy-meta-methoxybenzaldehyde, vanillin and its phenol sulfonate condensation product have met with only partial success and pyrophosphate zinc plating baths containing these aldehydes have not attained commercial acceptance. Similarly, I have found some other carbonyl compounds of aldehyde and ketone types have some beneficial effect on the pyrophosphate bath, but they also fail to provide an acceptable bright and uniformly smooth electrodeposit of zinc with good low current density coverage.

I have discovered that a small amount of an organic compound, hereafter referred to as a carrier, selected from the group consisting of (a) bis [sulfonaphthyl] methane; (b) naphthalene derivatives that contain substituents selected from the group consisting of sulfonic acids and their alkali metal salts, hydroxyl, amino, and imino radicals; (c) benzene derivatives containing the substituents selected from the group consisting of sulfonic acids and their salts with alkali metal and ammonium, alkyl and imino radicals, and (d) allyl sulfonic acid and its salts with alkali metals, when incorporated into a pyrophosphate zinc plating bath in combination with a carbonyl compound of the aldehyde and the ketone types will increase greatly the brightness and the uniformity of the zinc deposit. The low current density coverage of the bath also is improved, and the resultant electrodeposit of zinc shows a reduction in roughness.

According to this invention a preferred process for producing bright zinc deposits comprises electrodepositing zinc from an aqueous alkaline pyrophosphate solution containing at least one zinc salt in which there is dissolved from about 0.5 to about 5.0 grams per liter of a carrier selected from the group previously stated, and from about 0.025 to about 0.2 gram per liter of a carbonyl compound selected from the group consisting of aldehydes and ketones.

While the specific carriers of this invention may be used successfully at any concentration within the broad range stated above, it is generally preferable to employ them in a concentration from about 0.9 to about 1.6 grams per liter. Also it is preferred to employ the carbonyl compound at a concentration in the range from about 0.05 to about 0.1 gram per liter. I have found that the maxi-

2

mum brightness of the deposit is not obtained when the concentration of the carbonyl compound is too low. A high concentration of carbonyl compound, on the other hand, decreases the low current density coverage.

5 No specific procedure is required in adding the carrier to the plating bath. For the carbonyl compound, it is often most convenient to incorporate it in the bath in the form of dilute aqueous solution. For additives having higher carbonyl concentrations, basic aqueous solutions containing alkali metal hydroxide may be used. The short shelf life of this solution, however, requires that it be freshly prepared. For a solution having longer shelf life, the carbonyl compounds may be dissolved in the form of an aqueous-alcoholic solution.

10 Table I sets forth examples of the carriers that have been used successfully in the process of this invention.

TABLE I

- (a) bis [sulfonaphthyl] methane
- (b) naphthalene derivatives:
  - 2,6 naphthalene-disulfonic acid
  - 8 amino, 1 naphthalene, sulfonic acid
  - 6,6' imino bis-(1 naphthol-3) sulfonic acid
  - 2 naphthol-6,8 disulfonic acid
  - 2,3 dihydroxy-6 naphthalene sulfonate, sodium salt
  - 1,5 dihydroxy naphthalene
  - 1,4 naphthalene diol
- (c) benzene derivatives:
  - benzene monosulfonate, sodium salt
  - benzene sulfonamide
  - sodium toluene sulfonate
  - O-sulfonylbenzimidazole
- (d) sodium allyl sulfonate

35 Any of the carbonyl compounds of the aldehydes and ketone types which cooperate effectively with the carriers of this invention may be used in combination with the carriers of this invention in carrying out this process. I have found the carbonyl compounds that are effective have a structural formula selected from the group consisting of



45 wherein R is selected from the group consisting of hydrogen, alkyl, aryl and heterocyclic oxygen and sulfur radicals, and R' and R'' are selected from the group consisting of alkyl and aryl radicals. Both the alkyl and the aryl radicals in R, R' and R'' may contain substituents such as alkoxy or hydroxy radicals. Table II sets forth the carbonyl compounds that have been used successfully in combination with the carriers of this invention.

TABLE II

### Aldehydes

- $\begin{array}{c} R \\ \backslash \\ C=O \\ / \\ R \end{array}$
- 60 m-Hydroxy benzaldehyde
- p-Hydroxy benzaldehyde
- Piperonal
- o-Hydroxy benzaldehyde
- Veratraldehyde
- Benzaldehyde
- B-methoxy propionaldehyde
- Furfural
- Glyceraldehyde
- Anisaldehyde
- Salicylaldehyde propyl sulfone
- Ethyl vanillin
- Thiophene-2-aldehyde



In carrying out the process of this invention the optimum operating conditions such as the pH, the temperature, and the current density may vary depending upon the bath composition and the object being plated. In general, good bright zinc deposits can be obtained only within a specific range of operating conditions. For example, when the pH is much above the desired range, the zinc deposit loses its brightness, and when the pH is too low, the current efficiency decreases. Similarly, increasing the temperature reduces the brightness of the electrodeposit of zinc, but raises maximum current density that may be used before roughness occurs. Increasing the temperature also decreases the cathode current efficiency. Table III sets forth the range of the bath compositions and the operation conditions suitable for the process of this invention. The preferred compositions and conditions also are stated.

TABLE III

|                                               | Range       | Preferred   |
|-----------------------------------------------|-------------|-------------|
| Zinc Metal Concentration g./liter             | 10-60       | 20-30       |
| $\text{P}_2\text{O}_7/\text{Zn}$ Weight Ratio | 6.5:1-8.0:1 | 7.0:1-8.0:1 |
| pH                                            | 10.5-12.0   | 11.0        |
| $^{\circ}\text{C}$                            | 40-55       | 45-47       |
| Current Density, ASF                          | 2-40        | 4-20        |
| Carrier g./liter                              | 0.5-5.0     | 0.9-1.6     |
| Carbonyl Compound g./liter                    | 0.025-0.2   | 0.05-0.1    |

Vigorous but uniform agitation of the plating bath, which can be provided either by a mechanical or an air agitator is desirable during the electrodeposition. The agitation permits the use of higher plating current densities on the part being plated.

It is important during the plating operation that the metallic contamination should be eliminated to insure a bright metallic deposit. Metallic contamination from foreign metallic ions such as cadmium, copper and lead is the most troublesome. Conventional purification methods should be used to eliminate such metallic contami-

nation. Organic contamination may also be eliminated by circulating this pyrophosphate solution through activated carbon or other types of exchange or absorption media.

Although a number of combinations of carbonyl compounds can be used in connection with the carriers, as described previously, I find the combination of aldehyde, particularly the furfural and bis [sulfonaphthyl] methane gives excellent results in reduction of roughness, increase of brightness and increase of low current density coverage, at the same time offering the possibility of economical operation.

Following are examples of the process of this invention. In each of these examples a typical pyrophosphate plating bath having the following basic composition was used:

|                                                                            |               |       |
|----------------------------------------------------------------------------|---------------|-------|
| Zn as $\text{Zn}_2\text{P}_2\text{O}_7 \cdot \text{XH}_2\text{O}$ (31% Zn) | -----g./liter | 81    |
| $\text{K}_4\text{P}_2\text{O}_7$                                           | -----do       | 290   |
| Total $\text{P}_2\text{O}_7$                                               | -----do       | 188   |
| $\text{P}_2\text{O}_7/\text{Zn}$ weight ratio                              | -----         | 7.5:1 |

The pH of the bath was about 11 in all the cases and the temperature of the bath was maintained around 45° C. Plating operations in each example were carried out in an air agitated Hull test cell so the effect of a wide range of current densities could be observed. The zinc deposit in each example was plated on a Hull panel measuring 2½" x 3½" with 1 ampere current per panel for a period of 10 minutes.

The examples are used for the purpose of illustrating this invention and the synergistic effect of the carrier in combination with the carbonyl compounds. In the examples a Hull panel was plated first in the basic solution without the additives and then for each set of additives illustrated in the examples, two panels were plated, of which one was plated with the bath containing only one additive and the second panel was plated in accordance with the process of this invention. The resultant panels were compared by visual examination of the zinc deposits on the panels in both the high current density areas which were represented by one half of each Hull panel, and the low current density areas, which were represented by the remaining half of each panel. The back coverage which indicates the throwing power of the panel also was examined visually. The results are recorded in Table IV which shows the synergistic effects of various carbonyl compounds of the aldehyde and ketone types used in combination with a carrier, bis [sulfonaphthyl] methane.

TABLE IV

| Example | Additive                               |                                           | Visual Inspection and Comparison                                                  |                                                                      |                                           |
|---------|----------------------------------------|-------------------------------------------|-----------------------------------------------------------------------------------|----------------------------------------------------------------------|-------------------------------------------|
|         | Carbon Compound                        | Carrier                                   | High Current Density Area                                                         | Low Current Density Area                                             | Back Coverage                             |
| 1-----  |                                        |                                           | Coarse type of roughness; fine grained and semibright; color of the deposit dark. | Coarse grained and dull; uniform deposit.                            | Poor, major portion of the back unplated. |
| 2-----  | m-hydroxy benzaldehyde 0.75 g./liter.  |                                           | Roughness reduced; deposit bright and metallic.                                   | Fine grained and semibright; color of the deposit dark; freaky.      | Incomplete coverage.                      |
|         |                                        | Bis [sulfonaphthyl] methane 1.2 g./liter. | Roughness reduced, deposit bright and metallic.                                   | Smooth and bright deposit.                                           | Excellent coverage.                       |
|         |                                        |                                           | Roughness reduced; hazy bright deposit; non-uniform.                              | Deposit dull and non-uniform.                                        | Poor, major portion of the back unplated. |
| 3-----  | p-hydroxy benzaldehyde, 0.25 g./liter. | Bis [sulfonaphthyl] methane 1.2 g./liter. | Deposit bright and metallic...                                                    | Deposit bright and fine grained; improved uniformity of the deposit. | Excellent coverage.                       |
|         |                                        |                                           | Roughness; hazy bright deposit.                                                   | Fine grained; semibright; non-uniform.                               | Incomplete coverage.                      |
|         |                                        |                                           | Deposit bright and metallic...                                                    | Deposit bright and metallic; uniform.                                | Excellent coverage.                       |
| 4-----  | Piperonal 0.25 g./liter.               | Bis [sulfonaphthyl] methane 1.2 g./liter. | Roughness reduced; hazy bright deposit; non-uniform.                              | Coarse grained dull deposit; non-uniform.                            | Poor coverage.                            |
|         |                                        |                                           | Roughness reduced; hazy bright deposit; improved uniformity.                      | Improved brightness and uniformity.                                  | Excellent coverage.                       |
|         |                                        |                                           |                                                                                   |                                                                      |                                           |
| 5-----  | O-hydroxy benzaldehyde 0.05 g./liter.  | Bis [sulfonaphthyl] methane 1.2 g./liter. |                                                                                   |                                                                      |                                           |

TABLE IV—Continued

| Example | Additive                                       |                                           | Visual Inspection and Comparison                               |                                                              |                      |
|---------|------------------------------------------------|-------------------------------------------|----------------------------------------------------------------|--------------------------------------------------------------|----------------------|
|         | Carbon Compound                                | Carrier                                   | High Current Density Area                                      | Low Current Density Area                                     | Back Coverage        |
| 6       | Veratraldehyde 0.1 g./liter.                   | -----                                     | Roughness; hazy bright deposit.                                | Deposit bright and metallic; skipping and freaky.            | Incomplete coverage. |
|         |                                                | Bis [sulfonaphthyl] methane 1.2 g./liter. | Deposit bright and metallic.                                   | Deposit bright and metallic.                                 | Excellent coverage.  |
| 7       | Benzaldehyde 0.4 g./liter.                     | -----                                     | Roughness; hazy bright deposit; non-uniform.                   | Fine grained, semibright deposit; non-uniform.               | Incomplete coverage. |
|         |                                                | Bis [sulfonaphthyl] methane 1.2 g./liter. | Roughness; hazy bright deposit.                                | Brightness improved.                                         | Excellent coverage.  |
| 8       | B-methoxy Propionaldehyde 0.6 g./liter.        | -----                                     | Roughness; hazy bright deposit; non-uniform.                   | Coarse grained, dull deposit; non-uniform.                   | Incomplete coverage. |
|         |                                                | Bis [sulfonaphthyl] methane 1.2 g./liter. | Roughness; hazy bright deposit; non-uniform.                   | Improved in brightness and uniformity.                       | Excellent coverage.  |
| 9       | Furfural 0.1 g./liter.                         | -----                                     | Roughness reduced; fine grained, semibright deposit.           | Dull.                                                        | Poor coverage.       |
|         |                                                | Bis [sulfonaphthyl] methane 1.2 g./liter. | Fine grained; semibright deposit.                              | Fine grained; semibright deposit.                            | Excellent coverage.  |
| 10      | Glyceraldehyde, 0.1 g./liter.                  | -----                                     | Roughness, bright and metallic deposit; skipping; non-uniform. | Fine grained, semibright deposit.                            | Incomplete coverage. |
|         |                                                | Bis [sulfonaphthyl] methane 1.2 g./liter. | Roughness, bright and metallic deposit; skipping; non-uniform. | Fine grained, semibright deposit.                            | Excellent coverage.  |
| 11      | Anisaldehyde, 0.6 g./liter.                    | -----                                     | Roughness, hazy bright deposit.                                | Hazy bright deposit; non-uniform; skipping.                  | Poor coverage.       |
|         |                                                | Bis [sulfonaphthyl] methane 1.2 g./liter. | Roughness; deposit bright and metallic.                        | Deposit bright and metallic.                                 | Incomplete coverage. |
| 12      | Salicylaldehyde Propyl Sulfone, 0.05 g./liter. | -----                                     | Roughness reduced; deposit bright and metallic.                | Fine grained, semibright deposit, skipping; non-uniform.     | Incomplete coverage. |
|         |                                                | Bis [sulfonaphthyl] methane 1.2 g./liter. | Roughness reduced; deposit bright and metallic.                | The brightness improved; uniform.                            | Excellent coverage.  |
| 13      | Ethyl-Vanillin, 0.4 g./liter.                  | -----                                     | Roughness; hazy bright deposit.                                | Fine grained, semibright deposit; non-uniform.               | Incomplete coverage. |
|         |                                                | Bis [sulfonaphthyl] methane 1.2 g./liter. | Roughness; hazy bright deposit.                                | Improved in brightness.                                      | Excellent coverage.  |
| 14      | Thiophene-2-aldehyde 0.2 g./liter.             | -----                                     | Roughness; hazy bright deposit.                                | Dull.                                                        | Incomplete coverage. |
|         |                                                | Bis [sulfonaphthyl] methane 1.2 g./liter. | Roughness; hazy bright deposit.                                | Hazy bright deposit.                                         | Excellent coverage.  |
| 15      | Acetylacetone 4 ml./liter 5% solution.         | -----                                     | Roughness reduced; hazy bright deposit.                        | Fine grained, semibright deposit; color of the deposit dark. | Incomplete coverage. |
|         |                                                | Bis [sulfonaphthyl] methane 1.2 g./liter. | Roughness reduced; hazy bright deposit.                        | Deposit bright and metallic.                                 | Excellent coverage.  |

Similarly, the other carriers of this invention combine synergistically with a carbonyl compound of the aldehyde and ketone types to provide improvements in the brightness, uniformity and the low current density coverage of the electrodeposited zinc. Following are additional examples of the relative effects of these carriers on the zinc deposit when they are used alone or in combination with a carbonyl compound. The basic solutions and the operating conditions used in these examples are the same as those used in the previous examples.

#### Example 16

Two grams per liter of 8 amino, 1 naphthalene sulfonic acid were dissolved in the basic pyrophosphate solution. Zinc was electrodeposited onto a Hull panel. After the plating was completed, 0.1 gram per liter of furfural was added to the solution containing the carrier and a similar Hull panel was electrodeposited from this solution. These two plates were visually compared. It was found that the panel plated in accordance with the invention was brighter, more uniform and had better back coverage.

#### Examples 17-22

Similar to Example 16 except that 6,6'-imino bis-(1 naphthol-3) sulfonic acid; 2 naphthol-6,8 disulfonic acid;

2,6 naphthalene-disulfonic acid; 2,3- dihydroxy-6 naphthalene sulfonate (sodium salt); 1,5 dihydroxy naphthalene and 1,4 naphthalene diol were used separately as carriers in each example. When the two panels in each example were compared visually, the one plated in accordance with the process of this invention was either brighter, more uniform or had better back coverage.

#### Examples 23-26

60 Similar to the above examples except that benzene monosulfonate (sodium salt), having a concentration of 0.4 gram per liter was used as the carrier. The two panels plated were again compared visually and the one plated in accordance with the process of this invention was superior to the one plated in the solution containing only the carrier.

#### Example 27

Similar to the other examples except that 0.2 gram per liter of sodium allyl sulfonate was used as the carrier. The result was similar to those of the above examples.

From the examples given, the synergism between carriers of the type disclosed and carbonyl compounds, aldehydes or ketones, in pyrophosphate plating solutions is made apparent by the improvement in the characteristics of the electrodeposited zinc.

I claim:

1. The process for producing bright zinc deposits which comprises electroplating zinc from an aqueous alkaline pyrophosphate solution containing at least one zinc salt in which there is dissolved from about 0.5 to about 5.0 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.025 to about 0.2 gram per liter of a carbonyl compound having a structural formula selected from the group consisting of



wherein R is selected from the group consisting of hydrogen, alkyl, aryl and heterocyclic oxygen and sulfur radicals, and R' and R'' are selected from the group consisting of alkyl and aryl radicals.

2. The process for producing bright zinc deposits which comprises electrodepositing zinc from an aqueous alkaline pyrophosphate solution containing at least one zinc salt in which there is dissolved from about 0.5 to about 5.0 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.025 to about 0.2 gram per liter of an aldehyde having a structural formula



wherein R is selected from the group consisting of hydrogen, alkyl, aryl and heterocyclic oxygen and sulfur radicals.

3. The process for producing bright zinc deposits which comprises electrodepositing zinc from an aqueous alkaline pyrophosphate solution containing at least one zinc salt in which there is dissolved from about 0.5 to about 5.0 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.025 to about 0.2 gram per liter of a ketone having a structural formula



wherein R' and R'' each is selected from the group consisting of alkyl and aryl radicals.

4. The process for producing bright zinc deposits which comprises electrodepositing zinc from an aqueous alkaline pyrophosphate solution containing at least one zinc salt in which there is dissolved from about 0.9 to 1.6 grams per liter of a carrier selected from the group consisting of (a) bis [sulfonaphthyl] methane, (b) naph-

thalene derivatives that contain substituents selected from the group consisting of sulfonic acids and their alkali metal salts, hydroxyl, amino and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.05 to 0.1 gram per liter of a carbonyl compound having a structural formula selected from the group consisting of



wherein R is selected from the group consisting of hydrogen, alkyl, aryl and heterocyclic oxygen and sulfur radicals, and R' and R'' are selected from the group consisting of alkyl and aryl radicals.

5. The process for producing bright zinc deposits which comprises electrodepositing zinc from an aqueous alkaline pyrophosphate solution at a temperature ranging from about 40° C. to about 50° C., said solution containing 10 to 60 grams per liter of zinc which provides a pyrophosphate radical ( $P_2O_7$ ) to zinc weight ratio of 6.5 to 1 to 8.0 to 1 and a pH in the range from 10.5 to 12.0, in said solution there is dissolved from about 0.5 to about 5.0 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino, and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.025 to about 0.2 gram per liter of a carbonyl compound having a structural formula selected from the group consisting of



wherein R is selected from the group consisting of hydrogen, alkyl, aryl and heterocyclic oxygen and sulfur radicals, and R' and R'' are selected from the group consisting of alkyl and aryl radicals.

6. The process for producing bright zinc deposits which comprises electrodepositing zinc from an aqueous alkaline pyrophosphate solution at a temperature ranging from about 40° to about 50° C., said solution containing 20 to 30 grams per liter of zinc which provides a pyrophosphate radical ( $P_2O_7$ ) to zinc weight ratio of 7.0 to 1 to 8.0 to 1 and a pH of about 11.0, in said solution there is dissolved from about 0.9 to about 1.6 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino, and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.05 to about 0.1 gram per liter of a carbonyl compound having a structural formula selected from the group consisting of



wherein R is selected from the group consisting of hydrogen, alkyl, aryl and heterocyclic oxygen and sulfur radicals, and R' and R'' are selected from the group consisting of alkyl and aryl radicals.

7. The process for producing bright zinc deposits which comprises electrodepositing zinc from an aqueous alkaline pyrophosphate solution at a temperature ranging from about 40° C. to about 50° C., said solution containing 10 to 60 grams per liter of zinc which provides a pyrophosphate radical ( $P_2O_7$ ) to zinc weight ratio of 6.5 to 1 to 8.0 to 1 and a pH in the range from 10.5 to 12.0, in said solution there is dissolved from about 0.5 to about 5.0 grams per liter of bis [sulfonaphthyl] methane, and from about 0.025 to about 0.2 gram per liter of a ketone a structural formula



wherein R' and R'' each is selected from the group consisting of alkyl and aryl radicals.

8. The process for producing bright zinc deposits which comprises electrodepositing zinc from an aqueous alkaline pyrophosphate solution at a temperature ranging from about 40° C. to about 50° C., said solution containing 10 to 60 grams per liter of zinc which provides a pyrophosphate radical ( $P_2O_7$ ) to zinc weight ratio of 6.5 to 1 to 8.0 to 1 and a pH in the range from 10.5 to 12.0, in said solution there is dissolved from about 0.5 to about 5.0 grams per liter of bis [sulfonaphthyl] methane, and from about 0.025 to about 0.2 gram per liter of an aldehyde having a structural formula



wherein R is selected from the group consisting of hydrogen, alkyl, aryl and heterocyclic oxygen and sulfur radicals.

9. The process of claim 8 wherein about 0.9 to 1.6 grams per liter of said bis [sulfonaphthyl] methane is dissolved in said solution, and the concentration of said dissolved aldehyde is from 0.05 to 0.1 gram per liter.

10. The process of claim 9 wherein the aldehyde is furfural aldehyde.

11. A bright zinc plating bath comprising an aqueous alkaline pyrophosphate solution containing about 10 to 60 grams per liter of zinc which provides a pyrophosphate radical ( $P_2O_7$ ) to zinc weight ratio of 6.5 to 1 to 8.0 to 1 and a pH in the range from 10.5 to 12.0, about 0.5 to about 5.0 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and from about 0.025 to about 0.2 gram per liter of a carbonyl compound having a structural formula selected from the group consisting of



wherein R is selected from the group consisting of hydrogen, alkyl, aryl and heterocyclic oxygen and sulfur radicals, and R' and R'' are selected from the group consisting of alkyl and aryl radicals.

12. A bright zinc plating bath comprising an aqueous alkaline pyrophosphate solution containing about 20 to 30 grams per liter of zinc which provides a pyrophosphate radical ( $P_2O_7$ ) to zinc weight ratio of from about 7.0 to 1 to 8.0 to 1, about 0.9 to 1.6 grams per liter of a carrier selected from the group consisting of (a) bis [sulfonaphthyl] methane, (b) naphthalene derivatives that contain substituents selected from the group consisting of sulfonic acids and their alkali metal salts, hydroxyl, amino, and imino radicals, (c) benzene derivatives containing substituents selected from the group consisting of sulfonic acids and their salts with alkali metal and ammonium, alkyl and imino radicals, and (d) allyl sulfonic acid and its salts with alkali metals, and about 0.05 to 0.1 gram per liter of a carbonyl compound selected from the group consisting of



wherein R is selected from the group consisting of hydrogen, alkyl, aryl and heterocyclic oxygen and sulfur radicals, and R' and R'' are selected from the group consisting of alkyl and aryl radicals.

13. A bright zinc plating bath comprising an aqueous alkaline pyrophosphate solution containing at least one zinc salt, about 0.5 to about 5.0 grams per liter of bis [sulfonaphthyl] methane, and from about 0.025 to about 0.2 gram per liter of an aldehyde having a structural formula



wherein R is selected from the group consisting of hydrogen, alkyl, aryl and heterocyclic oxygen and sulfur radicals.

14. A bright zinc plating bath comprising an aqueous alkaline pyrophosphate solution containing about 10 to 60 grams per liter of zinc which provides a pyrophosphate radical ( $P_2O_7$ ) to zinc weight ratio of from about 10.5 to about 12.0, about 0.5 to 5.0 grams per liter of bis [sulfonaphthyl] methane and about 0.025 to 0.2 gram per liter of an aldehyde having a structural formula of



wherein R is selected from the group consisting of hydrogen, alkyl, aryl and heterocyclic oxygen and sulfur.

15. A bright zinc plating bath of claim 14 wherein said aldehyde is furfural aldehyde.

#### References Cited by the Examiner

#### UNITED STATES PATENTS

|    |           |         |                |          |
|----|-----------|---------|----------------|----------|
| 60 | 2,101,581 | 12/1937 | Henricks       | 204-55   |
|    | 2,488,246 | 11/1949 | Stareck et al. | 204-55   |
|    | 2,529,700 | 11/1950 | Lowe et al.    | 204-55 X |
|    | 3,049,942 | 6/1962  | Cox et al.     | 204-55 X |
| 65 | 3,088,884 | 5/1963  | Passal         | 204-55   |

JOHN H. MACK, Primary Examiner.

G. KAPLAN, Assistant Examiner.